

Sept. 14, 1937.

H. DREYFUS

2,092,803

MANUFACTURE OF TEXTILE MATERIALS

Filed Nov. 1, 1933

FIG. 1



FIG. 2



FIG. 3



FIG. 4



Inventor:  
Henry Dreyfus  
by  
Iseltzer and Belforrier  
Attorneys

## UNITED STATES PATENT OFFICE

2,092,803

## MANUFACTURE OF TEXTILE MATERIALS

Henry Dreyfus, London, England

Application November 1, 1933, Serial No. 696,184  
In Great Britain November 10, 1932

2 Claims. (Cl. 19—1)

This invention relates to the manufacture of textile materials, and in particular to yarns having a basis of continuous filaments, but having the appearance of spun yarn, that is yarn made from staple fibre.

In the manufacture of spun yarn from artificial fibres, the usual practice is to cut continuous artificial filaments or waste filaments into comparatively short lengths, for example of 1½ to 2 inches or more to produce a staple of similar length to cotton fibres or of 4, 7, 9, 12 inches or more to produce a staple somewhat similar in length to wool, and then subject the staple fibres produced alone or mixed with other natural or artificial fibres of suitable length to a series of operations appropriate to the length of the fibre, such operations being similar to those accorded to natural fibres such as cotton or wool, including opening, carding, drawing and spinning. These operations represent considerable expense in the production of such yarns, since they involve a relatively slow transformation of the initial fibrous material to a finished yarn.

It is possible, however, to effect the direct conversion of continuous filament yarn into spun yarn by subjecting the filament bundle to a sufficient tension to effect breakage of the filament and the production of a mass of fibres of substantially uniform length.

It has been found, however, that in relying on the extension of the filaments beyond their breaking point to transform the filaments into staple lengths, the consequent reduction in extensibility is somewhat disadvantageous in the final product, for, notwithstanding the fact that the product consists of discontinuous lengths instead of continuous lengths as in the bundle from which it was produced, the relatively low extensibility of the separate fibres results in the product having an elasticity which may be so low as to limit the applicability of the yarn for many textile purposes.

It has now been found, however, that the elongation of the spun yarn can be restored at least partially by a suitable conditioning treatment applied at any convenient stage after the conversion of the continuous filament yarn into the staple fibre product. Thus, for example, the twisted product may be subjected to the action of steam or to any suitable agent or treatment by means of which shrinkage and/or softening of the stretched fibres is brought about. This treatment may be effected after the final degree of twist has been imparted, and even after two or more of the spun yarns have been doubled to-

gether, or it may be effected at an intermediate stage of the twisting. For example, after twisting by means of a flyer spindle (conveniently continuously with the conversion of the filaments into staple lengths), the relatively lightly twisted yarn may be steamed or otherwise conditioned and thereafter further twisted or doubled. If desired the conditioning may be effected two or more times conveniently between different twisting operations.

The shrinking or softening treatment is particularly applicable in the production of spun yarns from continuous filaments of cellulose acetate or other organic derivatives of cellulose, but may be applied to the production of spun yarns from all kinds of continuous or staple fibre filaments, such as viscose, nitrocellulose and cuprammonium filaments.

While the conditioning treatment may be applied to the spun yarns or fibres of which the yarns are being made while they are travelling, it is convenient to effect the treatment while the material is wound into packages produced continuously with the conversion of the filaments into staple fibres, or packages produced by rewinding, e. g. hanks. Thus, these packages may be placed in a cabinet for a period and there subjected to the action of steam or any other conditioning agent. Such packages may consist of completely spun yarn, or they may consist of an intermediate product such as a sliver or roving, which is subsequently to be submitted to further operations, for example drawing and spinning. The material may indeed be submitted to treatment more than once. Thus it may be treated as a roving, and again as a finished yarn.

Where yarns are to be treated in the form of wound packages, steps may be taken to prevent the supports on which the packages are carried from constraining the yarn and preventing it from shrinking. It will be understood that the shrinkage of a package of yarns involves a reduction in diameter throughout the package, and the removal of constraint enables this reduction to have free play irrespective of the support upon which the yarn is wound to form a package. Where a relatively large package of yarn such as a cone, cheese or like package of yarn or roving is being treated, it is preferable that the material should be slackly wound on the core, that is, wound under a low tension or under no tension, so that the looseness of the package may be taken up when the yarn or roving on the package is caused to shrink. Alternatively, in the case of cones of yarn, a conical former having a rela-

tively large semi-vertical angle, e. g. 15°, or 17½° or more, may be employed, so that the yarn slips slightly on the former towards the apex thereof. Furthermore, a support may be used which is itself capable of reduction in diameter and susceptible of being compressed by the shrinking of the yarn or roving wound upon it. Thus, for example, the package support may consist of a piece of sheet material, such as a thin and springy metal sheet, bent into the form of a cylinder or cone, the edges of the sheet overlapping to form a support which is capable of reduction in diameter by the sliding of one edge of the sheet over the other. A package support of this form may be employed as the sole support for the package or may be provided with any suitable reinforcement which still permits of its reduction in size. Thus for example, in the formation of the package, the sheet may be bent around a former and the yarn may be wound thereon, while for the conditioning treatment of the package, the package with its metal sheet support may be removed from the winding former and placed upon a slightly smaller former, which, while supporting the package, permits a reduction in diameter of the package and of the metal sheet cylinder on which it is carried. In order to facilitate the conditioning treatment, the sheet of material on which the package is wound may be perforated to render it permeable to the agents employed in the shrinking operation.

Small packages of yarn such as cops, as employed in weaving, may be treated in a similar manner. Thus, they may be wound, preferably by a ring spinning operation, which may be effected continuously with the breaking of the continuous filaments, on cores capable of being reduced in diameter. The package so formed is then subjected to conditioning treatment, the thin sheet core being either the sole support of the package or being carried on a former of smaller size than the spindle upon which it was fitted while the package was wound. The thin sheet material forming the basis of the package may either comprise a sheet twisted once into a cylinder or it may comprise a long ribbon wound helically around the spindle of the ring or like twisting device to form a basis for the package during the operation of twisting and packaging.

As is indicated above, while steam or other conditioning medium may be applied to the spun yarn or intermediate product while it is travelling, it is convenient to effect the treatment while the yarn is wound on bobbins, for example on bobbins produced at the flyer spindle continuously with the conversion of the filaments. Thus, these bobbins may be placed in a cabinet for a period, and there subjected to the action 60 of steam.

Instead of steam, shrinkage and/or softening may be effected by means of aqueous liquids such as soap solutions, or even water. As other liquid agents which are especially suitable for bringing about shrinkage and/or softening of cellulose acetate or other cellulose derivative filaments may be mentioned acetic acid, formic acid, lactic acid, diacetone alcohol, acetone, the ethers, including the cyclic ethers, esters and ether-esters 65 of olefine and polyolefine glycols, for instance the mono- and di-methyl and ethyl ethers of ethylene glycol, glycol mono-acetate, methyl glycol mono-acetate, the mono-methyl and ethyl ethers of propylene glycol, the mono-ethyl ether 70 of diethylene glycol, dioxane, methylene ethylene

dioxide and the homologues and substitution products of these cyclic ethers, phenols, mono-, di- and tri-acetins, ethyl lactate, diethyl tartrate and the like, methylene chloride, ethylene chloride, chloroform, tetrachlorethane, dichloroethylene, ethyl acetate and like latent solvents for the cellulose derivatives, either alone or preferably modified as regards their action on the material by the addition of suitable diluents, as, for example, water, benzene, toluene, xylene or 10 other cyclic hydrocarbons, benzine, petrol ether, kerosene or other hydrocarbons of the aliphatic or petroleum series, carbon tetrachloride, trichloroethylene, perchloroethylene and other chlorinated or halogenated compounds which are inert 15 or comparatively inert towards the cellulose derivative. Solvent action on the material should be regulated in order to ensure that no substantial cementation of fibre to fibre takes place.

The conditioning agent may be applied in liquid form, e. g. in a scouring operation or by forcing it through the yarn wound on perforated tubes, or as a vapour, and may be removed in any suitable manner, e. g. by washing, centrifuging, evaporation, or any combination of these 25 methods. Thus for example, the whole treatment may be carried out in a hydro extractor, a number of large packages such as cones or cheeses or of smaller packages such as cops being placed in the extractor and treated for the 30 desired time with the liquid conditioning agent, which is then removed by centrifuging. This operation may be followed by a washing operation, the material being dried or partially dried 35 by a further centrifuging.

By way of example some forms of package supports which may be used for the purposes of the present invention are illustrated in the accompanying drawing in which:—

Figure 1 is a sectional view of a cross-wound 40 cone of yarn, and

Figures 2, 3 and 4 show a pim of yarn together with the means employed for carrying it.

In Figure 1 the yarn 5 is wound upon a package support 6 consisting of a sheet of metal 45 bent in the form of a cone, the edges 7 of the sheet overlapping. The package support 6 is carried upon a former 8 during winding, and for conditioning the yarn 5 is removed from the former 8 and placed upon a smaller former which 50 will allow the edges 7 of the package support 6 to slide over one another so that the yarn 5 may contract.

Figure 2 shows a spindle 10 carried in a bearing 11 and driven by means of a whorl 12. The spindle 10 is suitably shaped to carry a pim tube as shown in Figure 3, the pim being built by suitable traversing as the yarn is being twisted and wound. The pim tube 13 consists of a flexible 60 strip helically wound over the spindle 10, the edges of the strip overlapping as at 14. The yarn is wound on as shown at 15. In order to submit the yarn 5 to shrinking treatment the package is removed from the spindle 10 and placed upon a former 16 which, being smaller in diameter than the spindle 10, allows the pim tube 13 and the 65 yarn 5 to contract, the pim tube yielding under the shrinking action of the yarn.

The following are examples of modes in which the invention may be carried out:—

#### Example 1

A yarn consisting of staple lengths of cellulose acetate filament, produced by breaking continuous filaments, is wound in the form of a cone of 75

1/2 lb. weight on a support consisting of a sheet of thin springy metal twisted about a conical former, as described with reference to Fig. 1. The package on its sheet metal support is removed from the former and immersed in live steam for six hours. After this treatment the package is ready to be used, e. g. in a knitting operation, or for rewinding into smaller packages.

5 *Example 2*

10 A number of pirns of the yarn described in Example 1, wound on tubes consisting of spirally wound strips of sheet metal as described above with reference to Figs. 2, 3 and 4, are placed in a 15 centrifuge, and there treated with a solution of 50% by volume of methylene chloride in benzene at 15° C. The treating liquid is removed by centrifuging, and the pirns are washed with water, and partly dried by further centrifuging. After 20 stoving to complete the drying, the pirns are fit for use in a weaving operation.

What I claim and desire to secure by Letters Patent is:—

1. Process for the production of staple fibre

yarn from continuous filaments, said process comprising associating continuous filaments together with at least a slight twist, converting said continuous filaments into staple lengths by extending them to breaking point, winding the material into a package upon a support adapted to yield to shrinkage of the material thereon, and submitting the package to a shrinking operation to restore at least in part the extensibility lost by the material in the breaking operation.

5 2. Process for the production of staple fibre 10 yarn from continuous filaments, said process comprising associating continuous filaments together with at least a slight twist, converting said continuous filaments into staple lengths by extending them to breaking point, winding the material into a package upon a support comprising sheet material having free overlapping edges 15 and submitting the package so formed to a shrinking operation to restore at least in part the extensibility lost by the material in the breaking operation, the package support yielding to the shrinking of the material.

20 HENRY DREYFUS.